

## UNITED STATES PATENT OFFICE

2,230,000

## POLYVINYL CHLORIDE COMPOSITION AND SHEETS

Otto Hauffe and Wilhelm Wehr, Eilenburg, Germany, assignors to Deutsche Celluloid-Fabrik, Eilenburg, Germany, a corporation of Germany

No Drawing. Application April 18, 1936, Serial No. 75,241. In Germany April 20, 1935

5 Claims. (Cl. 260—42)

Our present invention relates to the manufacture of sheets from polyvinylchloride and more particularly to the manufacture of sheets from after-chlorinated polyvinylchloride.

5 One of its objects is to provide a process of producing improved sheets from after-chlorinated polyvinylchloride. Another object is the improved sheets of after-chlorinated polyvinylchloride. Further objects will be seen from the 10 detailed specification following hereafter.

In making sheets, foils, films, plastic masses and the like from cellulose derivatives or synthetic highly polymeric bodies with the aid of easily volatile solvents or alone by a heat treatment, it is usual to add one or more sparingly volatile solvents, so-called softening agents, for the purpose of obtaining a material which can be rolled. While in the case of plastic masses having a cellulose derivative basis, such an addition of a softening agent does in fact lead to an improvement, not only during the rolling but also in respect of the properties of the final product, in the case of synthetic highly polymeric bodies of the vinyl-group, particularly polyvinylchloride, after-chlorinated polyvinylchloride and mixed polymerizes of the chloride with acrylic acid derivatives, there is, indeed, a good effect experienced in the rolling operation but in respect of the properties of the finished sheet the 20 direct opposite is the case; thus, for example, the softening point, the mechanical strength and the dielectric properties are so far diminished that it is not possible to apply the sheet. Without the addition of a softening agent, however, sheets 25 of polyvinylchloride are too brittle and the after-chlorinated polyvinylchloride is practically incapable of being rolled; there are obtained merely uneven, shriveled, fragmentary pieces which are of no use.

According to this invention it has been found that after-chlorinated polyvinylchloride can be rolled by adding to the material polyvinylchloride instead of the hitherto usual softening agents. The addition of polyvinylchloride to the after-chlorinated polyvinylchloride may be between 10 and 95 per cent of the final product. Instead of polyvinylchloride there may also be used polystyrene. In this manner there are obtained without trouble, by rolling, coherent, completely smooth, not shriveled sheets of any thickness by means of thermal plasticizing. It has also been found that by rolling these materials together the mechanical properties of the polyvinylchloride are much improved. Whereas a 55 sheet of polyvinylchloride of 0.12 mm. thickness

shows in particular no measurable tensile strength, a sheet of similar thickness made from polyvinylchloride and after-chlorinated polyvinylchloride, in the proportion of 1:1, shows a tensile strength of 6 to 7 kg. per sq. mm. and an extension of 25 to 30 per cent in the longitudinal direction and 5 to 6 per cent. in the transverse direction. The dielectric properties of the sheet produced by rolling the polyvinylchloride and after-chlorinated polyvinylchloride 10 in the same operation are in no way affected disadvantageously; whereas hitherto the softening point has been strongly depressed even by a small percentage addition of a softening agent, the softening point of the after-chlorinated 15 polyvinylchloride is not affected by the non-chlorinated polyvinylchloride added for the purpose of facilitating the rolling operation. An addition of, for example, 20 per cent of phthalic acid ester to after-chlorinated polyvinylchloride 20 mainly for the purpose of rendering the material capable of being rolled, produces a sheet having a softening point of about 35 to 40° C., so that the sheet is quite useless for further application. If, however, the rolling of the same 25 after-chlorinated polyvinylchloride is facilitated by addition of non-chlorinated polyvinylchloride, for instance, in the ratio 1:1, there is obtained a sheet having a softening point of 77 to 30 80° C. Besides the mechanical strength the softening point has directly a preponderating importance in the working up of the polymeride into useful objects of any kind.

It must be regarded as a surprising advance in the art of plastic masses made from a basis 35 of synthetic polymerizes that, contrary to all expectation, by the rolling together of products which alone are not capable of being rolled or can be rolled only with great difficulty, such as after-chlorinated polyvinylchloride, and a very 40 brittle polymerize, the rolling of the product is facilitated on the one hand and on the other hand the mechanical strength of the material is improved without depressing its softening point.

45 What we claim is:

1. A composition adapted to form strong, smooth, supple sheets having high insulating power and a high softening point upon hot rolling thereof in the absence of solvents, consisting of a uniform mixture of after-chlorinated 50 polyvinylchloride and from 10 to 95 per cent by weight of the mixture of a vinyl polymer selected from the class consisting of polyvinylchloride and polystyrene.

2. A composition as defined in claim 1, where- 55

in the said two components of the mixture are present in about equal parts by weight.

3. Smooth, strong, supple sheets of high insulating power and a high softening point consisting of a uniform mixture of after-chlorinated polyvinyl chloride and from 10 to 95 per cent by weight of the mixture of a vinyl polymer selected from the class consisting of polyvinyl chloride and polystyrene.
- 10 4. Sheets as defined in claim 3, wherein the said two components thereof are present in about equal parts by weight.

5. Smooth sheets having a thickness of about .12 mm. consisting of a uniform mixture of about equal parts by weight of after-chlorinated polyvinyl chloride and polyvinyl chloride, said sheets having a tensile strength of 6 to 7 kgs. per square millimeter and an extensibility of 25 to 30 per cent in the longitudinal direction and 5 to 6 per cent in the transverse direction, and a high softening point and insulating power.

10

OTTO HAUFFE.  
WILHELM WEHR.